

## UNITED STATES PATENT OFFICE

WALTER MIEG, OF OPLADEN, AND RUDOLF MARIA HEIDENREICH, OF LEVERKUSEN-ON-THE-RHINE, GERMANY, ASSIGNEES TO GENERAL ANILINE WORKS, INC., OF NEW YORK, N. Y., A CORPORATION OF DELAWARE

## PROCESS FOR DYEING AND PRINTING TEXTILE FIBERS

No Drawing. Application filed June 18, 1930, Serial No. 462,138, and in Germany June 19, 1929.

The present invention relates to new indigoid vat dyestuff preparations and to the dyeing and printing of textile fibers with these preparations.

5 According to the present invention esters of indigoid vat dyestuffs corresponding to the probable general formula:



wherein R represents the radical of an indigoid dyestuff containing an indole ring system, n stands for one of the numbers 1 or 2 and wherein the CO-group is attached to the nitrogen atom of the indole ring system of R, obtainable according to the process described in U. S. application Ser. No. 379,879 filed 20th July 1929, are fixed on textile fibers, for example, on cotton fiber for instance by slop-padding or printing, on wool by acid dyeing or by any other known means. The acid amides of the above formula are obtainable by reacting upon the indigoid vat dyestuff containing an indole ring system with a benzoic acid sulfo halide in the presence of pyridine or a homologue thereof under substantially anhydrous conditions at a 20 temperature between about 80° C. and the boiling point of the reaction mixture, until a test portion is completely soluble in water. The ester of the indigoid vat dyestuff fixed upon the fiber is treated with alkaline agents whereby the ester is split off wholly or partly according to the quantity of alkali used. It is evident, that for wholly saponifying the ester at least the calculated amount of an alkaline agent is to be employed, but in practical work an excess of the alkaline agent will advantageously be used. For example, by printing on cotton the acid amide obtainable from indigo and benzoic acid meta sulfochloride as described above, steaming the printing in the Mather-Platt apparatus and then drawing it through a bath, containing a small quantity of free alkali, for a short time, a bright indigo printing is obtained. In a similar manner indigo dyeings are obtained by impregnating (slop-pad-

ding) cotton with the acid amide, steaming in the Mather-Platt and developing the dyeing with dilute alkali. In the same manner as indigo itself other indigoid dyestuffs can be applied to the fiber in the form of their esters. Dyeings can be obtained on wool by dyeing the ester in the presence of formic acid or sulfuric acid and then treating the dyeing for a short time with dilute alkali, or with copper acetate solution.

55 In contradistinction to the said sulfuric acid esters of vat dyestuffs, the so-called indigosols, which can only be developed in acid solution, the development can take place in the present case by means of alkaline agents.

60 The invention is further illustrated by the following examples, without being restricted thereto:

Example 1.—Cotton is printed with a dyestuff paste prepared according to the following directions:

41-43 parts of water  
6-4 parts by weight of the dyestuff ester obtainable by reacting upon indigo with benzoic acid-meta-sulfochloride in the presence of pyridine at a temperature of about 100-110° C.  
3 parts by weight of thioglycol  
50 parts by weight of thickening K (neutral starch tragacanth thickening.)  
100 parts by weight of paste.

75 This printing is steamed for 10 minutes in a Mather-Platt apparatus, developed by a short immersion (1/2 minute) at 45° C. into a bath, containing 50 grams of common salt and 50 ccs. of caustic soda solution of 36° Bé. per liter. The printing is then acidified and soaped in the customary manner. A clear printing of indigo is thus obtained, 80 possessing a rather better fastness to boiling than the customary indigo printings.

85 Example 2.—Cotton is slop-padded in the customary manner with an approximately 4-6% solution of the indigo acid amide of Example 1, to which some tragacanth has been added. After drying and passing for 10 minutes through a Mather-Platt apparatus, developing of the printings is performed as described in Example 1.

*Example 3.*—The acid amide of Example 1 is dyed on wool within some 1-1½ hours from a bath, which has been rendered acid with about 5% by weight of formic acid or 5 sulfuric acid, the dye bath containing 4% of dyestuff, calculated on the quantity of fiber to be dyed. Then the dyeing is developed on the fiber by a short treatment with a little alkali, whereby the original 10 violet dyeing of the fiber becomes blue. Alternatively the dyeing can also be developed by treating it for about 10 minutes at 55° C. with 250 ccs. of a 1% copper acetate filled up with water to 1½ liters.

15 We claim:—

1. Process which comprises impregnating textile fibers with an ester of an indigoid vat dyestuff having in its free form the probable formula:

20



25 wherein R represents the radical of an indigoid vat dyestuff containing an indole ring system, n stands for one of the numbers 1 or 2 and wherein the CO-group is attached to the nitrogen atom of the indole ring system 30 and treating the impregnated fiber with an alkali.

2. Process which comprises impregnating textile fibers with an ester of an indigoid vat dyestuff having in its free form the probable 35 formula:

40



45

and treating the impregnated fiber with an alkali.

3. Process which comprises printing cotton with a dyestuff paste having incorporated therewith a compound corresponding in its free form to the probable formula:

55



60

steaming the printing in a Mather-Platt apparatus, developing it in a bath containing

caustic soda solution, acidifying and soaping.

In testimony whereof, we affix our signatures.

WALTER MIEG.

RUDOLF MARIA HEIDENREICH.

70

75

80

85

90

95

100

105

110

115

120

125

130